

# United States Patent [19]

Knuppel et al.

[11] 3,773,496

[45] Nov. 20, 1973

[54] **PROCESS FOR PRODUCING CHROME STEELS AND A CONVERTER FOR CARRYING OUT THE PROCESS**

[75] Inventors: **Helmut Knuppel; Karl Brotzmann; Hans Georg Fassbinder**, all of Sulzbach-Rosenberg Hutte, Germany

[73] Assignee: **Eisenwerk-Gesellschaft Maximilianshutte mbH, Sulzbach-Rosenberg Hutte, Germany**

[22] Filed: **Feb. 18, 1971**

[21] Appl. No.: **116,447**

[30] **Foreign Application Priority Data**

Feb. 18, 1970 Germany ..... P 20 07 373.8

[52] **U.S. Cl.** ..... 75/60, 75/49, 75/52, 75/130.5

[51] **Int. Cl.** ..... C21c 7/08, C21c 7/10

[58] **Field of Search** ..... 75/51, 52, 59, 60, 75/49, 130.5

[56] **References Cited**

UNITED STATES PATENTS

|           |         |              |         |
|-----------|---------|--------------|---------|
| 3,594,155 | 7/1971  | Ramachandran | 75/60   |
| 3,252,790 | 5/1966  | Krivosfy     | 75/60   |
| 3,282,679 | 11/1966 | Richter      | 75/52   |
| 2,068,785 | 1/1937  | Bain et al.  | 75/49 X |

|           |         |                  |            |
|-----------|---------|------------------|------------|
| 2,093,666 | 9/1937  | Vogt .....       | 75/60      |
| 3,336,132 | 8/1967  | McCoy .....      | 75/49      |
| 3,507,642 | 4/1970  | Shaw .....       | 75/130.5 X |
| 3,198,624 | 8/1965  | Bell et al. .... | 75/130.5 X |
| 3,420,657 | 1/1969  | Hansen .....     | 75/130.5 X |
| 2,855,293 | 10/1958 | Savard .....     | 75/60      |

FOREIGN PATENTS OR APPLICATIONS

|           |         |                     |       |
|-----------|---------|---------------------|-------|
| 1,450,718 | 7/1966  | France .....        | 75/60 |
| 861,238   | 2/1961  | Great Britain ..... | 75/52 |
| 882,676   | 11/1961 | Great Britain ..... | 75/60 |

Primary Examiner—L. Dewayne Rutledge

Assistant Examiner—Peter D. Rosenberg

Attorney—Lawrence I. Field

[57]

**ABSTRACT**

Process of producing chrome steels of a chromium content of about 16 to 30 percent and low carbon and nitrogen contents. According to the process, a pig iron charge having a high chromium content and a carbon content of from 2 to 7 percent is refined by blowing with very pure oxygen under reduced pressure conditions, the oxygen being introduced into the melt below the level of the melt. The process is applicable to both ferritic and austenitic chrome steel production.

The application also discloses a novel bottom-blown converter construction for carrying out the refining procedure.

13 Claims, 1 Drawing Figure

Patented Nov. 20, 1973

3,773,496



INVENTORS  
HELMUT KNÜPPEL, KARL BROTMANN  
and HANS GEORG FASSBINDER

BY *Torin and McGahey*

Attorneys

**PROCESS FOR PRODUCING CHROME STEELS  
AND A CONVERTER FOR CARRYING OUT THE  
PROCESS**

**FIELD OF INVENTION**

The invention is concerned with a process for producing chrome steels of a chromium content of 16-30 percent and having low carbon and nitrogen contents.

While the invention is particularly applicable to the production of ferritic chrome steels of the indicated kind and will thus, in the following, primarily be described in connection with ferritic chrome steels, the invention can also be used for the production of austenitic steels.

**BACKGROUND INFORMATION AND PRIOR ART**

Ferritic chrome steels having a chromium content of between 15-30% and extremely low carbon and nitrogen contents exhibit superior forming properties and ductility. Further, such steels have excellent corrosion resistance and exhibit superior weldability, particularly if the steels are alloyed with molybdenum. In order to obtain steels with the indicated characteristics, the sum total of the carbon and nitrogen contents should be below 0.015% or should at least not exceed that value to any significant extent.

It is common practice to remove the carbon from the heat or melt by refining with oxygen. This, however, results in considerable difficulties since in the oxygen refining of chromium-containing melts, the chromium tends to be oxidized while, on the other hand, the nitrogen content of the melt is not sufficiently decreased. The reason for the oxidation of the chromium during the oxygen refining and the high chromium losses resulting therefrom resides in the high oxygen affinity of the chromium. The desired lowering of the nitrogen content is not achieved because the melt absorbs nitrogen from the refining gas and the atmosphere. Further, as is well known in this art, chromium increases the solubility of nitrogen so that the high chromium content in the melt is apt to raise the nitrogen content. In top blowing oxygen refining processes, wherein the oxygen is thus supplied from the top, the increase in nitrogen is also due to the fact that the oxygen jet or stream which emanates from the blowing or jetting lance at high speed results in a suction action, so that air or atmospheric nitrogen is sucked into the converter, thus introducing more nitrogen into the melt.

Numerous processes have been proposed for the purpose of producing chrome steels. All these prior art processes, however, require considerable technical expenditure or result in chrome steels which do not meet the requirements in respect to low carbon and nitrogen contents necessary for imparting to the steels the desired beneficial characteristics referred to.

Austrian Pat. No. 150,979 discloses, for example, a process for decarburizing ferro-chrome melts wherein a chromium containing melt of a carbon content of about 1% is charged into a vacuum reactor and is refined with pure oxygen or a refining gas containing a high percentage of oxygen. Due to the displacement of the carbon-oxygen equilibrium in the vacuum, this procedure results in a reduction of the chromium losses caused by chromium oxidation. However, the necessary extremely low carbon content required in ferritic chrome steels cannot be obtained. Furthermore, in this

prior art procedure no measures are taken to prevent nitrogen pickup by the melt.

Another prior art process is disclosed in U.S. Pat. No. 2,993,780, which concerns a procedure for the production of low alloy steels. In this prior art procedure, a pig iron melt is first refined in customary manner to form steel, for example, according to the top blowing oxygen procedure, and after the slag removal, the depth of the bath is decreased by tilting the converter. Sub-atmospheric pressure conditions are at the same time applied and an inert gas is blown through the melt. This prior art procedure, however, is not concerned with the production of ferritic chrome steels and does not suggest any means for the purpose of achieving the extremely low carbon and nitrogen contents that are desired in ferritic chrome steels. This holds true although the carbon content of the melt is decreased during the blowing of inert gas, such as argon, under vacuum conditions.

20 A further process for decarburizing steel melts containing about 3-30% chromium is disclosed in U.S. Pat. No. 3,046,107. This process suggests that a decreasing amount of oxygen is introduced into the melt together with an inert gas at temperatures of about 1,400°-1,900°C. The purpose of the introduction of the oxygen and the inert gas is to reduce the chromium loss and to achieve a final carbon content of 0.07%. However, this process does not consider the nitrogen content of the steel, and the starting point for the process is a remelt or steel charge.

With a view to producing stainless steels with low carbon content and low nitrogen content, it has more recently been proposed to operate in an arc furnace. The procedure referred to thus suggests to melt in an arc furnace an iron charge containing up to 26% of chromium, up to 1% of carbon and up to 1% of silicon. The melt is subsequently, and in a separate reaction vessel, decarburized by blowing a mixture of oxygen and argon until the carbon content has been reduced to 0.010%.

All the prior art processes, including the ones referred to, have as primary purpose to keep as low as possible the chromium losses which occur during the decarburization of the chrome containing steels. This is achieved, on the one hand, by refining at relatively high temperatures and, on the other hand, by the use of a mixed gas consisting of oxygen and an inert gas, at least during a portion of the refining procedure. Further, in these prior art processes, the chromium, which unavoidably is oxidized during the blowing, is recovered for the melt by the addition of reducing agents such as, for example, silicon and/or aluminum. However, the nitrogen content has not been considered of particular importance in these processes, so that the nitrogen content of the customary chrome steels, dependent on the chromium content, usually is between 0.02 and 0.085%. For example, a chrome steel containing 9-11% of chromium, 2-8% of manganese, and 1-5% of nickel may customarily contain 0.07-0.08% nitrogen.

**SUMMARY OF THE INVENTION**

It is the primary object of the invention to propose a procedure which can be readily carried out on a large technical scale in economical manner and which results in the production of chrome steels, particularly ferritic chrome steels, of exceedingly low nitrogen content, thereby obtaining a chrome steel which has the desired

superior characteristics in respect to ductility and shaping or forming.

It is also an object of the invention to provide a process of the indicated kind which can be carried out with a minimum of expenditure and which results in a chrome steel of superior characteristics.

Generally it is an object of the invention to improve on the art of making chrome steels, both of ferritic and austenitic nature, as presently practiced.

Further, it is an object of the invention to provide a converter structure eminently suitable for carrying out the inventive procedure.

The solution of the inventive tasks is based on the realization that the desired low nitrogen content can be obtained in an economically feasible manner if the composition of the starting melt is chosen such, and the refining procedure is controlled in such a manner, that already during the decarburization with pure oxygen the nitrogen content of the melt is decreased to an extent which is far greater than the customary nitrogen removal which occurs as the result of blowing of pure oxygen.

Briefly, the invention provides that a pig iron or hot metal charge having a high chromium content and a carbon content of about 2-7% is refined under reduced pressure conditions by blowing very pure oxygen below the level of the melt, while,

The success of the inventive procedure is based on the fact that, due to the blowing with very pure oxygen under reduced pressure conditions, a very rapid decarburization is obtained resulting in a carbon content of extremely low values while, at the same time, nitrogen pickup from the refining gas and/or the ambient atmosphere is successfully prevented.

Of essential importance is the unusually high carbon content of the starting melt which leads to an intense CO formation during the refining. This intense CO formation is the cause for the considerable reduction of the nitrogen content already during the first refining phase. In this manner, nitrogen contents can be obtained which are considerably below the nitrogen values of a steel of comparable composition which has been refined in customary manner and subsequently has been degassed in a vacuum.

The carbon content of the starting melt is advantageously made dependent on the nitrogen content of the starting melt. For example, with a nitrogen content of 0.035% and at a pressure in the refining vessel of about 0.1 atm, the carbon content should initially be about 6 percent. Experiments have indicated in this context that the pressure above the melt during the refining should be the lower the lower the carbon content is of the original charge. Within a range of 2-6% carbon, it may be stated as a rule of thumb that the ratio of initial carbon content to absolute pressure which is 60 in the above example always be maintained. It is therefore recommended, considering an economical performance of the procedure, to start with a relatively high initial carbon content.

Considering that an extremely low nitrogen content is desired, the refining is advantageously performed with oxygen of a purity degree of 99.9% which, in addition to noble gases, may possibly contain not more than 10 ppm of nitrogen. The purity of the argon should be at least 99.95 and preferably 99.99 percent.

Practical experience has indicated that the carbon content, in spite of the high initial value, may be low

ered to 0.5% while the nitrogen content is at the same time decreased from about 0.035 to 0.010%. The decrease in carbon content as result of the refining, despite the initial high carbon content of the melt, does not result in any substantial chromium oxidation. Considering that a rapid decrease of the nitrogen and carbon contents is desired while, at the same time, avoiding substantial chromium slagging, the additional refining is advantageously performed with a mixture of oxygen and an inert gas which is essentially free of nitrogen. Such inert gas may, for example, be argon and/or hydrogen which facilitates the formation of CO bubbles in the melt. The proportion of inert gas in the oxygen may be gradually increased until the inert gas, at the end stage of the blowing, amounts to 90-100%.

The inventive procedure may be carried out particularly economically and advantageously in a bottom blown converter.

The various features of novelty which characterize the invention are pointed out with particularity in the claims annexed to and forming a part of this disclosure. For a better understanding of the invention, its operating advantages and specific objects attained by its use, reference should be had to the accompanying drawing and descriptive matter in which there is illustrated and described a preferred embodiment of the invention.

The single FIGURE of the drawings indicates a sectional view of a preferred embodiment of a converter suitable for carrying out the inventive procedure.

Referring now to the drawing, the converter shown therein consists of a steel shell 3 which is lined with a refractory lining 4. A bottom plate 5 is provided which supports the removable tuyere bottom 6. One half of the bottom 6, the lefthand side in the drawing, is traversed by a plurality of tuyeres or nozzles 7. Each nozzle consists of an inner tube 9 and an outer tube 11, the inner tubes 9 being all connected to a common oxygen line 8, while all the outer tubes 11 are connected to a common inert gas conduit or line 10. It will be noted that the nozzles or tuyeres are inclined relative to the longitudinal axis of the converter.

The mouth 12 of the converter is relatively small and is situated within a hood 13 which is placed on the converter and connected therewith in gas-tight manner.

The hood is provided with a vacuum tube 14 and communicates with a container 15 for receiving the alloying ingredients which, after opening of the slide valve 16, are charged from the container 15, without pressure decrease, into the converter. The container 15 with the slide 16 thus acts as a vacuum lock or sluice and the detachable hood 13 is connected with the converter shell in vacuum-tight manner. The converter shell 3 is preferably welded in vacuum-tight manner.

The converter is provided with a pouring hole 17 which, during the refining procedure, is closed by means of a closure or cap 18 in gas-tight manner. Contrary to the customary substantially cylindrically constructed converters, the converter here shown and particularly suitable for the inventive procedure is shaped approximating that of a sphere or ball. Such sphere-like converters are more suitable for the present invention.

Further, the filling degree of the converter should be lower than in the customary procedures. Thus, for example, if a 20-ton charge is customarily refined in a converter defining a space of 15 m<sup>3</sup>, then a converter to be used for refining a 20-ton charge in accordance with the inventive procedure should have about twice

the volume, to wit, about 30 m<sup>3</sup>. It is also important that the leak losses caused by uptight areas should not exceed 0.01 percent of the off-gases which are sucked off through the vacuum pipe 14.

In top blowing oxygen procedures difficulties occur due to the high temperature stresses to which the lance is subjected by the hood. These difficulties are successfully avoided in bottom blown converters. Further, in the instant bottom blown converter, the high degree of utilization of the blown oxygen and the negligible production of brown smoke make it possible to maintain the sub-atmospheric pressure conditions in the converter and the removal by suction of the reaction gases by means of a steam ejector pump, which does not require any preceding purification of the off-gases and which at the same time effectively washes out the dust components of the off-gases. The relatively small amounts of off-gases can be readily managed and may be discharged through an off-gas line of relatively small inner diameter of about 500 mm.

The invention will now be described by an example, it being understood, however, that this example is being given by way of illustration and not by way of limitation and that many changes may be effected without affecting in any way the scope and spirit of the appended claims.

#### EXAMPLE

This test was carried out in a converter of the kind shown in the drawing, having an interior space of 30 m<sup>3</sup>. The converter was charged with 20 tons of an alloyed pig iron charge containing 22% of chromium, 6% of carbon and 0.035% of nitrogen. The temperature was 1,450°C and blowing was effected for 20 minutes with 50 Nm<sup>3</sup>/min. of oxygen under simultaneous blowing of 3% of propane, calculated on the amount of blown oxygen. The propane was introduced through the annular space between the inner tubes and the associated outer tubes of the tuyeres. The carbon content of the melt amounted to 0.5% while the nitrogen content amounted to 0.010% after this first refining stage. The bath or melt temperature rose during this stage to 1,700°C. The melt could be replenished with about 4% of chrome ore, calculated on the weight of the melt. This was done by opening the slide 16 so that the chrome ore dropped into the converter from the container 15. The carbon removal and nitrogen removal was then continued by blowing an oxygen-argon mixture. During a further blowing period of 20 min., the argon portion which originally was 10%, when the carbon content was 0.5%, was gradually increased to 95%, while the carbon content in the melt decreased to 0.005%, and the pressure in the final phase of the refining was lowered to 10-20 mmHg. The propane supply was interrupted when the argon moiety of the blowing gas amounted to 50 percent and instead pure argon was used as shell gas. No significant wear of the tuyeres could be observed. The particular advantage of blowing with pure argon as shell gas during the final phase of the refining resides in the fact that the refined steel is characterized by an extremely low hydrogen content. Although during the second blowing phase the amount of the blown gas is decreased to 20 Nm<sup>3</sup>/min., a final carbon content of 0.005% and a final nitrogen content of 0.008% were obtained. With a view to preventing nitrogen pickup, both the emptying of the converter and

the pouring of the steel should be effected under protective gas atmosphere.

The starting chromium content of the melt may be lower than would be required in the light of the desired final chromium content. This is so because the high blowing temperature at the end of the first blowing stage renders it possible to add significant amounts of chromium ore at that time. Considering the significant increase of the solubility of nitrogen with increasing chromium content, the initial relatively low chromium content results correspondingly in a lower initial nitrogen content of the charge to be refined. In order to expedite and accelerate the reduction of the chromium ore, silicon and/or aluminum may at the same time be added to the converter as reduction agent.

According to a modification of the inventive procedure, the refining gas and/or the mixture of refining gas and inert gas may be admixed with lime in powder form. This results, surprisingly, in a particularly quiet blowing without the formation of foaming slag and metal splashing. This general advantage has a particularly favorable effect in the inventive converter construction since the problems caused by the sealing of the structure can be more readily solved. Further, due to the addition of lime, a satisfactory and early phosphorus and sulfur removal takes place. Accordingly, it is then also possible to use less expensive starting materials. If the initial phosphorus and sulfur contents are high, it may be required to operate with two slags. In experimental melts, the first slag was removed after about 3-10 min. and the refining procedure corresponding to the above example was continued and terminated under a second slag.

As previously stated, the invention is particularly suitable for the production of ferritic steels. However, austenitic steels may also be produced in accordance with the inventive procedure and in the inventive converter structure. However, in producing austenitic steels the requirements of the individual process steps need not be exactly adhered to. Thus, for example, it is sufficient if the pressure above the melt is in a range of 1-0.3 atm. The admixture of inert gas during the refining process may be increased toward the end of the procedure up to 100 percent.

What is claimed is:

1. A process for producing chrome steels in a refractory lined vessel with a chromium content of about 16-30% and of extremely low carbon and nitrogen contents, the sum of the carbon and nitrogen contents being not more than about 0.015% by weight, which comprises:

refining a molten pig iron charge having a high chromium content and an initial carbon content of about between 2-7% by introducing at least one stream of pure oxygen through at least one injector extending through the refractory lining of said vessel and having an opening communicating with the interior of the vessel below the surface of the molten charge and terminating at the exposed surface of the refractory lining;

protecting said injector and said refractory lining during introduction of oxygen into the molten metal while maintaining the opening of each such injector substantially unobstructed for the flow of fluid therefrom into the vessel by surrounding each such oxygen stream with a protective fluid containing hydrocarbon in an effective amount;

while maintaining a subatmospheric pressure over the melt, and continuing said refining until the total carbon and nitrogen content is below about 0.015% by weight.

2. A process as claimed in claim 1, wherein the chrome steel to be produced is of ferritic nature.

3. A process as claimed in claim 1, wherein, after an initial refining with oxygen, the oxygen is blown in admixture with an inert gas which is substantially free of nitrogen.

4. A process as claimed in claim 1, wherein an inert gas is admixed with the oxygen during a portion of the refining procedure.

5. A process as claimed in claim 1, wherein the oxygen which is blown into the melt is admixed with an inert gas after the carbon content of the melt has been reduced to about 0.5 percent.

6. A process as claimed in claim 1, wherein the blowing of the oxygen is effected, at least during a portion of the blowing procedure, in admixture with an inert gas, the amount of inert gas gradually increasing in the

8 mixture until it has reached a value of about 90-100 percent in the final stages of the refining procedure.

7. A process as claimed in claim 1, wherein the maximum amount of nitrogen in the oxygen is about 10 ppm.

8. A process as claimed in claim 3, wherein the maximum amount of nitrogen in the oxygen and the inert gas totals not more than 0.05 percent.

9. A process as claimed in claim 3, wherein the blowing is effected so that a portion of the inert gas surrounds the oxygen which is blown into the melt.

10. A process as claimed in claim 1, wherein the oxygen blown into the melt is surrounded by a veil of propane gas.

15 11. A process as claimed in claim 1, wherein the oxygen is admixed with powdered lime.

12. A process as claimed in claim 3, wherein the blowing gas mixture is admixed with powdered lime.

13. A process as claimed in claim 1, wherein the 20 charge is bottom blown.

\* \* \* \* \*

25

30

35

40

45

50

55

60

65